

## UNITED STATES PATENT OFFICE

FRITZ GRETER, OF BASEL, SWITZERLAND, ASSIGNOR TO THE FIRM OF SOCIETY OF CHEMICAL INDUSTRY IN BASLE, OF BASEL, SWITZERLAND

## PROCESS FOR DYEING SILK FAST TINTS

No Drawing. Application filed March 12, 1930, Serial No. 435,366, and in Switzerland March 16, 1929.

The present invention relates to a new process for dyeing silk fast tints. It comprises the dyeing process and the material dyed according to the new process.

5 The dyeing of silk in neutral or fatty soap baths is a process which comes increasingly to the fore in the silk dye-house.

It has now been found that complex metalliferous azo-dyestuffs which may contain several metals are excellently suitable for producing fast tints on silk in a bath the pH of which lies between 6.8 and 10. Particularly suitable for the process are among others those complex metal compounds which 10 are derived from azo-dyestuffs made by coupling diazo-compounds containing lake-forming groups and aminonaphthol compounds containing as many  $\text{SO}_3\text{H}$ -groups as naphthalene residues, which couple in ortho-position to the hydroxyl group, and which 15 may be substituted at the nitrogen atom. Such products are inter alia the aminonaphthol-mono sulfonic acids and their derivatives, such as the urea or the dinaphthyl derivatives of the 2:5:7-aminonaphthol sulfonic acid.

ing metals, such as aluminium, vanadium, chromium, manganese, iron, cobalt, nickel, copper, zinc, etc., as coming into consideration to produce these metalliferous dyestuffs.

The following examples illustrate the invention, the parts being by weight:

## Example 1

Silk is dyed with addition of 10-20 per cent of crystallized sodium sulfate, the goods being entered at 60° C. and the bath heated gradually to 80-85° C., whereupon dyeing is continued for  $\frac{3}{4}$  to 1 hour at this temperature.

## Example 2

Ordinary or loaded silk is dyed with addition of 1-2 grams of Marseilles soap per litre and 10-30 per cent of crystallized sodium sulfate, the goods being entered at 60° C. and the bath being heated gradually to 80-85° C. whereafter dyeing is continued for  $\frac{3}{4}$  to 1 hour at this temperature.

The following table gives some of the tints obtainable according to the present invention by dyeing in the manner described in Example 1 or 2.

| No. | Diazotizing component                                               | Coupling component                                                                                | Metal | Tint produced on loaded silk |
|-----|---------------------------------------------------------------------|---------------------------------------------------------------------------------------------------|-------|------------------------------|
| 30  | 2-amino-1-phenol-4:6-disulfonic acid                                | 2-amino-5-hydroxynaphthalene-7-sulfonic acid                                                      | Cu    | Bordeaux.                    |
| 2   | 2-amino-1-phenol-4:6-disulfonic acid and 4-chloro-2-amino-1-phenol. | 2-amino-5-hydroxynaphthalene-7-sulfonic acid                                                      | Cr+Cu | Do.                          |
| 3   | 5-nitro-2-amino-1-phenol                                            | 2-phenylamino-5-hydroxynaphthalene-7-sulfonic acid                                                | Cr    | Greenish-blue.               |
| 4   | Do                                                                  | do                                                                                                | Cr+Cu | Blue.                        |
| 5   | Do                                                                  | do                                                                                                | Cu    | Blue-violet.                 |
| 6   | Anthranilic acid                                                    | do                                                                                                | Cu    | Violet.                      |
| 7   | 4-chloro-2-amino-1-phenol                                           | 2-acetylamino-5-hydroxynaphthalene-7-sulfonic acid                                                | Cu    | Red-violet.                  |
| 8   | Dichloro-2-amino-1-phenol                                           | 2-benzoylamino-5-hydroxynaphthalene-7-sulfonic acid                                               | Cu    | Red-violet.                  |
| 9   | 5-nitro-2-amino-1-phenol                                            | do                                                                                                | Cr    | Green-gray.                  |
| 10  | 2 mol of 2-amino-1-phenol-4-sulfamide                               | 2,2'-dimaphthylamine-5,5'-dihydroxy-7,7'-disulfonic acid                                          | 2 Cu  | Violet.                      |
| 40  | 11 2 mol of 2-amino-1-phenol-4-sulfamide                            | Urea of 2-amino-5-hydroxynaphthalene-7-sulfonic acid                                              | Cr+Cu | Brown-violet.                |
| 12  | 12 2 mol of 4-chloro-2-amino-1-phenol                               | Azo-dyestuff from diazotized 2-amino-5-hydroxy- and 2-amino-5-hydroxynaphthalene-7-sulfonic acid. | Cr    | Grey.                        |
| 13  | 13 5-nitro-2-amino-1-phenol                                         | 1-amino-8-hydroxynaphthalene-4-sulfonic acid                                                      | Cu    | Green.                       |

45 Particularly chromium and copper are pointed out among the known complex-form-

There must be named also as suitable for the invention among others metal compounds

50

55

60

65

70

80

85

90

of dyestuffs obtained from the following diazo-components: diazotized 5-nitro-4-chloro-2-amino-1-phenol, 4-chloro-2-amino-1-phenol-6-sulfonic acid, 4-nitro-2-amino-1-phenol-6-sulfonic acid, 6-nitro-2-amino-1-phenol-4-sulfonic acid, picramic acid, para-aminosalicylic acid, and coupling components, namely: 2-methylamino-5-hydroxynaphthalene-7-sulfonic acid, 2(2'-methoxy)-phenylamino-5-hydroxynaphthalene-7-sulfonic acid, 2(2'-ethoxy)-phenylamino-5-hydroxynaphthalene-7-sulfonic acid, 2(2'-methoxy-4'-methyl)-phenylamino-5-hydroxynaphthalene-7-sulfonic acid, 2-benzylamino-5-hydroxynaphthalene-7-sulfonic acid, 2,2':4'-dichloro)-benzoylamino-5-hydroxynaphthalene-7-sulfonic acid, 2(3'-nitro)-benzoylamino-5-hydroxynaphthalene-7-sulfonic acid, 2-benzoylamino-8-hydroxynaphthalene-6-sulfonic acid, 2-amino-8-hydroxynaphthalene-6-sulfonic acid, 1-amino-8-hydroxynaphthalene-4-sulfonic acid, 1-benzoylamino-8-hydroxynaphthalene-4-sulfonic acid, 1-phenylamino-8-hydroxynaphthalene-4-sulfonic acid, 2-acetylamino-8-hydroxynaphthalene-6-sulfonic acid.

What I claim is:

1. A process for the production of fast tints on silk, consisting in treating silk in a bath the pH of which lies between 6.8 and 10, with complex metal compounds which are derived from azo-dyestuffs made from diazo-compounds containing lake-forming groups and aminonaphthol compounds containing as many  $\text{SO}_3\text{H}$ -groups as naphthalene residues, and which couple in ortho-position to the hydroxyl group.
2. A process for the production of fast tints on silk, consisting in treating silk in a bath the pH of which lies between 6.8 and 10, with compounds of complex metals the atomic weight of which lies between 52 and 64 which are derived from azo-dyestuffs made from ortho-hydroxy-diazo-components and aminonaphthol compounds containing as many  $\text{SO}_3\text{H}$ -groups as naphthalene residues, and which couple in ortho-position to the hydroxyl group.
3. A process for the production of fast tints on silk, consisting in treating silk in a bath the pH of which lies between 6.8 and 10, with compounds of complex metals the atomic weight of which lies between 52 and 64 which are derived from azo-dyestuffs made from ortho-hydroxy-diazo-components and amino-naphthol mono-sulfonic acids which couple in ortho-position to the hydroxyl groups.
4. A process for the production of fast tints on silk, consisting in treating silk in a bath the pH of which lies between 6.8 and 10, with compounds of complex metals the atomic weight of which lies between 52 and 64 which are derived from azo-dyestuffs made

from ortho-hydroxy-diazo-components and an aminonaphtholmono-sulfonic acid of the general formula



70

wherein R stands for H, alkyl, aryl, aralkyl or acetyl, y in one case stands for an OH-group and in the other case for a hydrogen atom, z in one case stands for an  $\text{SO}_3\text{H}$ -group and in the other case for a hydrogen atom, and in which the OH-groups and the  $\text{SO}_3\text{H}$ -group stand in meta-position to each other.

5. A process for the production of fast tints on silk, consisting in treating silk in a bath the pH of which lies between 6.8 and 10, with compounds of complex metals the atomic weight of which lies between 52 and 64 which are derived from azo-dyestuffs made from ortho-hydroxy-diazo-components and a 2-amino-5-hydroxynaphthalene-7-sulfonic acid of the general formula



95

wherein R means a hydrogen atom, aryl, alkyl or aralkyl.

6. A process for the production of fast tints on silk, consisting in treating silk in a bath the pH of which lies between 6.8 and 10, with compounds of chromium and copper which are derived from azo-dyestuffs made from ortho-hydroxy-diazo-components and a 2-amino-5-hydroxynaphthalene-7-sulfonic acid of the general formula



110

wherein R means a hydrogen atom, aryl or aralkyl.

7. A process for the production of fast tints on silk, consisting in treating silk in a fatty soap bath with compounds of chromium and copper which are derived from azo-dyestuffs made from ortho-hydroxy-diazo-components and a 2-amino-5-hydroxynaphthalene-7-sulfonic acid of the general formula



125

wherein R means a hydrogen atom or aryl.

8. A process for the production of fast

130

tints on silk, consisting in treating silk in a fatty soap bath with a chromium compound which is derived from an azo-dyestuff made from ortho-hydroxy-diazo-components and 5 2-amino-5-hydroxy-naphthalene-7-sulfonic acid of the formula

10



15 In witness whereof I have hereunto signed

my name this 28th day of February, 1930.

FRITZ GRETHER.

20

25

30

35

40

45

50

55

60

65